

## 1

3,079,211

## TREATMENT OF TANNED LEATHERS

Maxime Paquet, Route de Nice, Cuers (Var), France  
 No Drawing. Filed Sept. 28, 1959, Ser. No. 842,605  
 Claims priority, application France Mar. 23, 1956

19 Claims. (Cl. 8—94.21)

The present invention relates to the treatment of leathers tanned with zirconium based tanning baths, with a view to controlling their water absorbing properties as well as their permeability to air.

This is a continuation-in-part of my co-pending application Serial No. 641,458, filed February 21, 1957, now abandoned.

It has been found and verified since a number of years that tanning with zirconium, when properly conducted can produce leathers which are very resistant to wear and friction. However, such leathers have the serious drawback of absorbing too high quantities of water, which restricted their use. Various attempts have been made in different directions to decrease the said water absorption but such attempts have led either to a destruction of the favorable properties resulting from zirconium tanning, or to make the treated leathers impervious to air, and finally no satisfactory solution has been found.

The object of my invention is to provide zirconium tanned leathers the water absorption qualities of which are conveniently controlled without impairing their perviousness to air, or their resistance to wear.

I have found that if fibers of zirconium tanned leather are put in contact with higher fatty amines in proper conditions, the said amines form with the acid reacting, tanning zirconium compounds which are fixed on said fibers, highly water repellent compounds which are also solidly fixed on the fibers and which durably impart their water repellancy to the treated leather. It would seem that an inversion of electric charges occurs, although this is a mere supposition.

The fatty amines which are operative in my invention are the long chain primary amines derived from fatty acids, of the general formula  $R.NH_2$  in which R is an unsubstituted aliphatic chain having from 8 to 22 carbon atoms. Such amines may be considered as deriving from ammonia through replacement of one hydrogen atom by a fatty chain without any other substitution.

Appropriate amines are caprylylamine ( $C_8$ ), caprylamine ( $C_{10}$ ), laurylamine ( $C_{12}$ ), myristylamine ( $C_{14}$ ), palmytylamine ( $C_{16}$ ), stearylamine ( $C_{18}$ ), oleylamine ( $C_{18}$ ), arachidylamine ( $C_{20}$ ), behenylamine ( $C_{22}$ ) and the like, the above list not being limitative. The average molecule weights of said amines range from about 130 to about 320.

Although all the above amines give favorable results the best results are obtained with oleylamine or palmytylamine, and natural or artificial mixtures of various amines having 16 or 18 carbon atoms may be used satisfactorily in my invention. For example, I obtain good results with the mixture of oleylamine stearylamine and palmytylamine with a dominant proportion of oleylamine, as obtained when treating commercial fatty acids.

Generally speaking, I prefer using amines derived from unsaturated fatty acids such as oleic or linoleic acids, rather than amines deriving from saturated acids. However, mixtures containing both types of amines are suitable, and in fact often necessary when special detail effects are desired.

By commercial higher aliphatic or fatty amines, I mean herein products of the modern chemical industry obtained by treating with ammonia, fatty acids having  $C_8$  to  $C_{22}$  chains, whether alone or in natural mixtures, in liquid or gaseous phase, at a given temperature and in

## 2

suitable conditions. Intermediary products are thus obtained, to wit nitriles, which are thereafter hydrogenated to the commercial fatty amines used in my invention. The intermediary nitriles give no results in the method according to my invention.

The above defined amines are neither pure products, nor products which can be defined other than by their method of manufacture but the primary amines of the fatty acids employed are largely dominant, which is sufficient for my process.

It is neither recommended nor necessary to use more complicated amines than those above-mentioned, e.g. amines comprising multiple or conjugated linkages, no particular or favourable effects being obtained therewith.

Although the above defined amines alone are adapted to give the desired results, I have found that the diamines of the same above mentioned fatty acids, which diamines are obtained by similar methods and often in more or less great quantities at the same time as the primary amines also give satisfactory results and may be used in conjunction with said primary amines. Said diamines may be represented by the general formula:



in which R has the same meaning as above. The said diamines thus comprise both a primary amine group and a secondary amine group. Like the above mentioned primary fatty amines, they are strong bases and they have similar general properties with however a more pronounced polarity and a stronger cationic character.

It would appear that most of the commercial fatty amines, due to their method of preparation, contain more or less important quantities of such diamines.

All the above mentioned amines and diamines are solid or liquid according to the degree of saturation of the fatty chain, and to their molecular weight. They are insoluble in water and soluble in mineral oils, in hydrocarbons, more particularly when added with alcohol, in ethyl, methyl, isopropyl alcohols and the like, and in chlorinated solvents such as trichlorethylene, perchlorethylene or carbon tetrachloride. All said amines and diamines react with organic or mineral acids to give salts the properties of which largely depend on the acid which is used. Thus, most of the monoacids such as hydrochloric, acetic, formic, lactic acids and the like give water soluble salts. The chlorides are soluble in water and soluble in oils whereas the acetates and formates are soluble both in water and in hydrocarbons, as well as in chlorinated solvents.

Organic or mineral diacids of higher polyacids generally give salts which are insoluble in water and variously soluble in various solvents.

According to my invention, leathers must be treated by amines of the above mentioned type, which have been wholly or partly neutralized by an acid or acids, because of their strongly basic properties, the said neutralized amines being dissolved either in water or in organic solvents depending on the neutralizing acid and the results which it is desired to achieve.

I have found that the solutions in organic solvents should be preferred for the treatment of thick leathers, whereas aqueous solutions may be used for the treatment of thin or highly porous leathers.

More particularly for the treatment of thick or "heavy" zirconium tanned leathers, the amines or mixtures of amines and diamines are dissolved in an organic solvent or a mixture of such solvents, then neutralized by adding to said solution one or more convenient acids.

Preferred amines are oleylamine, linoleylamine, palmytylamine and stearylamine or mixtures thereof and the solvent should preferably be trichloroethylene or a hydrocarbon.

I have found that for neutralizing the amine or amines, tartaric acid should be used in a quantity equal to at least half the total quantity of acid which is necessary for complete neutralization. The said acid should be preferably added in powdered form, while stirring, to the amine solution maintained between 60 and 70° C. The reaction is exothermic and care should be taken to avoid a temperature rise above 80° C. which could result in an unfavorable transformation of amines into amides.

I have also found that part of the basicity of the amines may advantageously be neutralized by means of very weak acids such as phenic acid (phenol) or abietic acid (colophane).

The presence of such weak acids is useful even when the amines are completely neutralized by means of tartaric acid.

Tartaric acid may be in part replaced by citric, sulfuric, sulfurous or phosphoric acid. Cresol may be used instead of phenol and any other resin having an acid reaction instead of abietic acid.

I have furthermore found that the addition of a small quantity of boric acid to the tartaric acid substantially improves the results obtained. It seems that boro-tartaric acid is formed, which acts favorably as a catalyst of the various subsequent reactants in the presence of the fibers of leather tanned with zirconium.

Since the amines employed have a totally basic character which it is easy to estimate quantitatively, these amines should be neutralized by:

The tartaric acid (plus boric acid when so required) should be comprised between 50% and 100% of the quantities necessary for the total neutralization of the basicity of the amines;

The boric acid should amount to between 0 and 20% of the quantity of tartaric acid;

The phenol ( $C_6H_5OH$ ) or cresol should comprise between 10% and 50% of the total quantity of amines existing in the solution, this total being calculated in pure amines (according to their quantitative basicity);

The abietic acid should preferably comprise between 20% and 90% of the same total weight of the amines.

These solutions in trichlor-ethylene are stable at temperatures which do not exceed 75° C. They are characterised by a high fluidity, a high degree of penetration into the leather or other porous materials, and by their special properties of becoming fixed on products having an acid reaction.

For the treatment of heavy leathers tanned with zirconium, these solutions should be employed with a content of amines (calculated in pure amines) comprised between 3% and 15% of their weight.

The leathers tanned with zirconium or with mixed mineral tannings, brought to a pH value between 3.5 and 5.0, carefully washed and then dried or almost dried, are soaked for 10 to 40 minutes in the solution described above, maintained between 15° and 50° C., depending on the case, and then dried in air at a temperature not exceeding 40° C.

The results are improved by operating in a closed tank in which a certain depression is maintained, for example 30 cm. of mercury. The solvent may be recuperated by drying in an appropriate apparatus with or without vacuum.

The leathers thus treated and dried are already strongly water-repellent and can be used commercially in that state in certain cases. They have however generally been subjected to excessive dehydration, which modifies their properties and their appearance.

It has been found that it is useful to subject them to a controlled hydrolysis, during which they fix a small quantity of water and recover an average general humidity, which can be estimated by the usual method, comprised as required between 12% and 18%.

This hydrolysis is effected by soaking the leathers as treated above and dried for one hour or more, in a bath

5  
10  
15  
20  
25  
30  
35  
40  
45  
50  
55  
60  
65  
70  
75

of water maintained between 40° and 50° C. During the course of this operation, the appearance and colour of the leathers change completely and their water-repellent characteristics are considerably increased after they have again been dried.

To this bath of water, there may be added when so required, small quantities of particular reagents (for example various organic acids) so as to modify certain details relative to qualities and appearance.

The application of the invention is illustrated in the examples given in the following text. These examples are understood to be illustrative only, and the invention is in no way limited by the indications given therein.

#### Example 1

Heavy butts of cow leather are strongly tanned with zirconium following a standard method with a very acid pH value (about 1.5) and with about 6.5% of zirconium oxide calculated on the weight of leather butts in strips.

The completely tanned skins are rendered basic in a tanning bath up to a pH value of about 3.0 and are then neutralized in a fresh bath to a pH value of 4.0 to 4.5 and carefully washed.

If so desired, they are then rapidly surface-dyed by soaking for about one hour in a light bath of a vegetable tanning extract (for example chestnut) so as to obtain a pleasing appearance. The leathers are then allowed to drain, dried and then rolled. They give by analysis about 15% humidity.

At this stage, the leathers show a water absorption of 65% to 70% with the Kubelka apparatus in one hour, and have an excellent resistance to wear.

The leathers are then treated as below so as to render them water-repellent and to give them special qualities.

For this purpose, an impregnating solution A is made:

In 1200 kg. of trichlor-ethylene there is dissolved while heating to 60° C.: 100 kg. of commercial oleyl-amine containing 92 kg. of primary fatty amines composed of palmityamine 7 kg., stearyl-amine 4 kg. oleyl-amine 81 kg., the average molecular weight of these amines being 268. The estimation of the basicity showed that 29.6 kg. of pure tartaric acid would be necessary to obtain complete neutralization.

To this solution, kept at 60° C., there is slowly added: 25 kg. of tartaric acid and 2.5 kg. of boric acid, both these acids being in the form of powder.

After complete reaction, which requires about 12 hours, 28 kg. of phenol are added, followed by 47.5 kg. of colophane.

After leaving to rest for 3 days, this solution A is ready for use. There is thus available about 1400 kg. of a solution containing about 6.6% of oleyl-amine, 2% of phenol and 3.4% of colophane.

100 kg. of the zirconium leathers referred to above are soaked for 30 minutes in the impregnating solution A, maintained at 45° C.

The leathers are removed from the bath; after draining they weigh about 140 kg. (before drying). They have fixed about 2.7 kg. of fatty amines, or 2.7%.

The leathers are completely dried in air between 20° and 35° C., after which they give the following water absorption in the Kubelka apparatus:

9 to 10% in 1 hour  
16 to 18% in 3 hours  
34 to 38% in 24 hours

The impregnated and normally-dried leathers give on analysis a humidity content of 8 to 10%.

The gluing of these leathers with neoprene glues is possible, but necessitates very extensive carding of the surfaces.

#### Example 2

The leathers obtained by the treatment of Example 1 are again treated to give a hydrolysis. To this end, they are soaked for one and a half hours in a bath of water

## 5

held at 45° C., after which they are dried in air between 20° and 35° C.

After drying, their colour is much lighter and more uniform and their appearance is definitely more pleasing.

With the Kubelka apparatus, they give the following degrees of water absorption:

5 to 7% in 1 hour  
8 to 9% in 3 hours  
26 to 29% in 24 hours

When normally dried, these leathers give 14 to 16% humidity on analysis: they can readily be glued.

## Example 3

100 kg. of the same zirconium leathers are impregnated with the same solution A, but this operation is carried out in a suitable tank, in which is maintained a temperature of 45° C., and a depression of about 30 cm. of mercury. The period of impregnation is 25 minutes, after which the solution is evacuated and the leathers are left in the tank. The solvent is then evaporated in the tank itself, in which is maintained a depression of 10 to 20 cm. of mercury. After 40 minutes in a suitable apparatus, about 90% of the solvent used for the impregnation is recovered in this way.

The leathers are removed from the tank and completely dried in air at about 30° C.

After leaving to rest in this state, a hydrolysis treatment is made, as in Example 2 above, but with water at 45° C. to which there has been added 1 part in 10,000 of its weight of ethylene-diamine tetracetic acid. The leathers thus obtained and dried are of very light colour and pleasant appearance. It is found by analysis that they have fixed 3.5% of fatty amines and that they have an average humidity of 14 to 16%.

With the Kubelka apparatus, these leathers give greatly improved water-absorption characteristics as follows:

3 to 5% in 1 hour  
7 to 8% in 3 hours  
22 to 24% in 24 hours

These leathers can be glued perfectly and without any difficulty. Together with a very low water-absorption characteristic, they have an excellent and substantially increased resistance to wear together with mechanical, physical and chemical properties which are both new and very favorable, in particular exceptional resistance to pulling off, tearing and abrasion.

## Example 4

The same process is followed as for Example 3, but the impregnating solution employed is obtained with the following mixture:

Commercial oleyl-amine: 50%  
Commercial stearyl-diamine: 50%

For the neutralization of 100 kg. of this mixture, the quantity of tartaric acid is brought up to 29 kg., the other constituents remaining unchanged.

The impregnating operation and the hydrolysis process are the same as for Example 3.

The results obtained are also comparable with those obtained in Example 3, namely:

Similar water absorption characteristics;

The leathers are darker with a more greasy appearance;

The leathers are softer and more flexible;

The resistance to tearing is exceptionally high.

## Example 5

The same process is followed as in Example 3, but the impregnating solution is obtained by using the mixture of fatty amines resulting from the treatment of a

## 6

mixture of fatty acids from ordinary tallow. This mixture contains:

About 30% of palmityl-amine  
About 40% of oleyl-amine  
About 30% of stearyl-amine

The neutralization of the solution is obtained as in Example 3, the other constituents remaining unchanged.

10 The operation of impregnation and hydrolysis are effected in the same way as in Example 3.

The results obtained are closely similar to those described in Example 3, but the leathers are stiffer, their appearance is less pleasing, and the favorable effects of hydrolysis are reduced.

## Example 6

15 The same process is employed as for Example 3, but the impregnating solution is obtained by utilizing the mixture of fatty amines resulting from the treatment of the natural mixture of fatty acids in copra oils. This mixture gives on analysis the following approximate composition:

|                                   | Percent |
|-----------------------------------|---------|
| Caprylyl-amine (C <sub>8</sub> )  | 8       |
| Capryl-amine (C <sub>10</sub> )   | 9       |
| Lauryl-amine (C <sub>12</sub> )   | 47      |
| Myristyl-amine (C <sub>14</sub> ) | 18      |
| Palmityl-amine (C <sub>16</sub> ) | 8       |
| Stearyl-amine (C <sub>18</sub> )  | 5       |
| Oleyl-amine (C <sub>18</sub> )    | 5       |

20 The average molecular weight of these amines is 196. The neutralization of the solution is carried out as in Example 3, with the exception that 32 kg. of tartaric acid are added to 100 kg. of the above amines in solution; the other constituents remain unchanged.

25 The operations of impregnation and hydrolysis are the same as in Example 3.

30 The leathers obtained give the following water-absorption characteristics with the Kubelka apparatus:

40 12 to 15% in 1 hour  
18 to 20% in 3 hours  
36 to 42% in 24 hours

45 The water-repellent effects are definitely less than in the case of Example 3, but they will often be adequate. The leathers are flexible, light in colour and of very pleasant appearance.

## Example 7

50 The same process is followed as in Example 3, but the impregnating solution is obtained by employing the mixture of fatty amines resulting from the treatment of the fatty acids of hydrogenated tallow, which are thus saturated fatty acids.

55 This mixture of amines has the following approximate composition:

|                | Percent |
|----------------|---------|
| Palmityl-amine | 30      |
| Stearyl-amine  | 68      |
| Oleyl-amine    | 2       |

60 The average molecular weight of these amines is 265.

The neutralization of the solution is carried out as in Example 3, employing the same acids and the same other constituents.

65 The operations of impregnation and hydrolysis are also the same as those described in Example 3 and give similar results in respect of water absorption, but the leathers are firmer, darker in colour and have a less pleasing appearance. The favorable effects of hydrolysis are reduced and the leathers are more difficult to glue with standard neoprene glues.

## Example 8

70 The same process is followed as in Example 3, but the impregnating solution is obtained with a mixture of

Fatty amines derived from commercial fatty acids with 20 to 22 atoms of carbon.

This mixture has the following approximate composition:

|                              | Percent |
|------------------------------|---------|
| Arachidyl-amine ( $C_{20}$ ) | 56      |
| Behenyl-amine ( $C_{22}$ )   | 35      |
| Stearyl-amine ( $C_{18}$ )   | 9       |

The average molecular weight of these amines is about 310.

The neutralization of the solution is carried out as in Example 3, but only 20 kg. of tartaric acid are employed for 100 kg. of the above amines; the other constituents remain unchanged.

The operations of impregnation and hydrolysis are carried out in the same way as in Example 3. The leathers obtained are very firm, of dark appearance and their surface feels greasy to the touch. They are difficult to glue, but the water absorption properties are excellent. Leathers of this kind can have valuable features for certain particular cases.

The examples given above can be summarized by stating that the use in the process of the present invention of oleyl-amine and mixtures of oleyl-amine and linoleyl-amine (unsaturated fatty chains) give the most favorable results in the majority of the usual cases, but the other amines may produce leathers which have certain characteristics specially suitable for particular cases.

*Example 9.—Replacement of a Part of the Tartaric Acid in the Above Examples by Another Polyvalent Acid*

The same procedure is followed as in Example 3 above.

The impregnating solution is obtained with commercial oleyl-amine which gives by analysis the following composition:

|                | Percent |
|----------------|---------|
| Oleyl-amine    | 85      |
| Palmityl-amine | 10      |
| Stearyl-amine  | 5       |

The average molecular weight of the above amines is about 270.

The neutralization of the solution containing 100 kg. of these amines is carried out as in Example 3, except in that the following are added:

|               | Kg. |
|---------------|-----|
| Tartaric acid | 16  |
| Boric acid    | 2   |
| Citric acid   | 10  |

The above acids are in powder form.

The other constituents remain unchanged.

The operations of impregnation and hydrolysis are also the same as in Example 3. The leathers obtained have similar characteristics to those of the leathers of Example 3, with the following observations:

The water absorption percentages are higher;

The penetration of the amine compounds into the leather is less uniform, due to the greater viscosity of the impregnating solution;

The leathers have an excellent appearance.

From a large number of tests made by substituting another acid for part of the tartaric acid, the following conclusions have been reached:

The replacement of part of the tartaric acid by sulphuric acid, sulphurous acid, phosphoric acid and other polyvalent acids, taking account of their valency and their molecular weight, results in solutions the viscosity of which increases with the quantity of these acids employed, while the penetration into the leathers diminishes rapidly. On the other hand, the water-repellent effects are favorable.

The replacement of part of the tartaric acid by a monovalent acid-hydrochloric acid, acetic acid, formic acid, lactic acid, etc., rapidly results in excessive water absorption as measured with the Kubelka apparatus. This ef-

fect can be employed to regulate the water absorption to any value desired, according to the case.

*Example 10.—Influence of the Solvent Used*

The same procedure is followed as in the case of Example 3, the same amines, same operations of neutralization, and the same addition of the other constituents, but the 1200 kg. of trichlor-ethylene (impregnating solution A) are replaced by 750 kg. of ordinary benzene (density 0.9, boiling point 81° C.).

The operation of impregnation and hydrolysis are carried out as in Example 3.

The results obtained are in all respects very similar to those obtained with trichlor-ethylene employed as the solvent in Example 3, the conditions of recovery of the solvent and of drying being of course appropriate to the solvent and the necessary precautions being taken in view of its inflammability.

It has been found that the results obtained with these leathers, within the framework of the present invention, vary very little with the solvents employed, provided that the latter are taken from the family of chlorinated solvents (tetrachlor-ethylene, perchlor-ethylene, carbon tetrachloride, etc.), or from the family of hydrocarbon solvents (benzene, toluene, naphtha solvents, etc.).

The choice of the solvent from the above groups should be made by taking account of their solvent qualities for the amine compounds, of their physical properties (density, boiling point, speed of evaporation, etc.), of their facility of use and of recovery within the scope of their commercial utilization.

It has been found that alcohols can be employed as solvents, especially when another solvent is added, since generally speaking, the alcohols rapidly reduce the water-repellent properties of the leathers treated, resulting in water absorption percentages, as given by the Kubelka apparatus, which rapidly become excessive with increasing proportions of alcohol used as a solvent (ethyl alcohol, methyl alcohol, isopropyl alcohol, etc.).

I claim:

1. A method for imparting water repellency to leathers tanned with a zirconium based tanning bath, while maintaining high resistance to wear and high permeability to air, which comprises impregnating said leathers with a solution in an organic solvent of compounds selected from the group consisting of a higher aliphatic primary amine of the general formula  $R-NH_2$  and compounds selected from the group consisting of an amine of the general formula



in which R is an aliphatic chain comprising 8 to 22 carbon atoms and mixtures of said amines, said amines having been previously combined with tartaric acid in at least one-half the amount required to neutralize said amine, and thereafter hydrolyzing said leathers by soaking in water at a temperature between about 25 and 55° C., and drying said hydrolyzed leather in air.

2. A method as claimed in claim 1, in which the amine is commercial oleylamine.

3. A method as claimed in claim 1, in which the soaking solution is a solution of a mixture of amines derived from the fatty acids of copra oils, containing a major proportion of aliphatic chains containing 10, 12 and 14 carbon atoms.

4. A method as claimed in claim 1, in which the soaking solution is a solution of a mixture of primary fatty amines derived from the fatty acids of tallow having chains containing 16 and 18 carbon atoms, of which fatty acids about 40% are constituted by oleic acid.

5. A method as claimed in claim 1, in which is used a mixture of primary fatty amines derived from commercial oleic acid, said amines containing a proportion of at least 85% of oleyl-amine.

6. A method as claimed in claim 1, in which the soak-

ing solution is a solution of a mixture of primary fatty amines derived from hydrogenated tallow the predominating quantities in said amine mixture being constituted by stearyl-amine and palmityl-amine.

7. A method as claimed in claim 1, in which the soaking solution is a solution of a mixture of primary fatty amines having chains with 20 and 22 atoms of carbon, the preponderant quantities in said amine mixture being constituted by arachidyl-amine and behenyl-amine.

8. A method as claimed in claim 1, in which said impregnating solution comprises quantities of fatty amines comprised between 3% and 18% by weight, calculated in pure amines before neutralization.

9. A method as claimed in claim 1, in which to said impregnated solution are added the following:

10 to 40% of tartaric acid of the weight of the amines and diamines, calculated in pure amines or diamines; from 0 to 40% of phenol or cresol of the weight of the amines and diamines, calculated in pure amines or diamines; from 10 to 90% of colophane of the weight of the amines and diamines, calculated in pure amines or diamines; from 0 to 20% of boric acid, calculated on the weight of tartaric acid used.

10. A method as claimed in claim 1, in which the solvent employed for said soaking solution is a chlorinated solvent.

11. A method as claimed in claim 1, in which the solvent employed for said soaking solution is a hydrocarbon.

12. A method as claimed in claim 1, in which the solvent employed for said soaking solution contains at least one alcohol in a proportion not exceeding 50%.

13. A method as claimed in claim 1, in which part of the tartaric acid employed in said soaking solution is replaced by a polyvalent acid selected from the group consisting of citric acid, sulphuric acid, sulphurous acid, phosphoric acid, this substitution not exceeding 40% of the total quantity of acid necessary for the complete neutralization of said amines.

14. A method as claimed in claim 1, in which at least a part of the tartaric acid employed in said impregnating solution is replaced by a monovalent acid selected from the group consisting of hydrochloric acid, acetic acid, formic acid, lactic acid, this substitution not exceeding 25% of the quantity of acid necessary for the complete neutralization of said amines.

15. A method as claimed in claim 1, in which the water employed for the hydrolysis of said leathers is acidified by the addition of a small quantity of an acid.

16. A method as claimed in claim 15, in which said acid is ethylene-diamine tetracetic acid.

17. A method for imparting water repellency to leather tanned with a zirconium based tanning bath, while maintaining high resistance to wear and high permeability to air, which comprises impregnating said leathers with a solution in an organic solvent of compounds selected from the group consisting of a higher aliphatic primary amine having an aliphatic chain of 8 to 22 carbon atoms and mixtures of said amines and previously combined with tartaric acid in at least one-half the amount required to neutralize said amine, said solution also containing phenol and colophane and evaporating said solvent.

18. A method for imparting water repellency to leathers tanned with a zirconium based tanning bath, while maintaining high resistance to wear and high permeability to air, which comprises impregnating said leathers with a solution in an organic solvent of compounds selected from the group consisting of a higher aliphatic amine of the general formula



25 in which R is an aliphatic chain comprising 8 to 22 carbon atoms and mixtures of said amines, said amine having been previously combined with tartaric acid in at least one-half the amount required to neutralize said amine, said solution also containing phenol and colophane.

19. A method as claimed in claim 18, in which the soaking solution is a solution of a mixture of primary fatty amines and fatty diamines, said amines and diamines being constituted by fatty chains having from 12 to 20 atoms of carbon.

#### References Cited in the file of this patent

#### UNITED STATES PATENTS

40 2,343,920 Maxwell ----- Mar. 14, 1944  
2,868,833 Szabo et al. ----- Jan. 13, 1959

#### FOREIGN PATENTS

45 452,630 Great Britain ----- Aug. 21, 1936

#### OTHER REFERENCES

J.A.L.C.A., March 1959, page 178, vol. LIV, No. 3.